# EUROPEAN PATENT APPLICATION

(11) **EP 4 782 563 A1**
(43) Date of publication of application: **29.07.2026**
(21) Application number: 25153485.5
(22) Date of filing: 23.01.2025
(51) Int. Cl.: C22C 33/02, C22C 38/00, C22C 38/10, C22C 38/12, C22C 38/22, C22C 38/26, C22C 38/30

(54) **POWDER-METALLURGICAL CHROMIUM- AND NIOBIUM-CONTAINING STEEL AND METHOD OF MANUFACTURING THE SAME**

(71) Applicant: voestalpine BÖHLER Edelstahl GmbH & Co KG, 8605 Kapfenberg (AT)
(72) Inventor: ZUNKO, Horst, 8605 Kapfenberg (AT); FLUCH, Rainer, 8605 Kapfenberg (AT); GELDER, Siegfried, 8605 Kapfenberg (AT)
(74) Representative: Lambsdorff & Lange Patentanwälte Partnerschaft mbB

(57) **Abstract**

A powder-metallurgical steel consists of, in % in weight: C: 0.35% to 0.6%, N: 0.01% to 0.3%, Cr: 12% to 15%, Mo: 3% to 5.5%, Co: 1.6% to 5%, Nb: 1.2% to 1.75%, and optionally one or more of Si: less than 1.5%, Mn: less than 1.5%, W: less than 0.5%, Ni: less than 0.5%, Al: less than 0.3%, V: less than 1.0%, Ti: less than 1.0%, Ta: less than 0.5%, the balance being Fe and incidental impurities.

## Description

### Technical Field

This disclosure relates to a powder-metallurgical steel, and in particular to a powder-metallurgical chromium- and niobium-containing steel.

### Background

In specific technical areas, steels are required which exhibit a combination of high corrosion resistance and high hardness, while still providing good toughness for avoiding cracks or chipping during operation. For example, applications in plastics processing, e.g. injection molding or other plastic forming processes, and applications such as industrial blade materials or hand knives, particularly in the food industry, require highly corrosion-resistant steels with high hardness and wear resistance combined with good toughness and polishability.

An NbC-containing powder-metallurgical martensitic steel has been described by Hahn, Isabel, et al., "Novel Development of an NbC-Containing Powder-Metallurgical Martensitic Steel with Outstanding Tribocorrosion Resistance", steel research int., 2023, 94, 2200474, pages 1-7. This steel consists of a martensitic matrix with evenly dispersed Nb-rich monocarbides having a fraction in volume of 2.5 vol%. The fine dispersion of monocarbides increases the wear resistance, whereas high contents of chromium, molybdenum and nitrogen dissolved in the metal matrix exert a positive effect on the corrosion properties.

Powder-metallurgical production of Nb- and C-containing steels is difficult, because primary carbides, which form in an Nb- and C-containing melt during atomization, tend to agglomerate in the nozzle and clog it. Therefore, to avoid clogging, a conventional manufacturing route for producing powder-metallurgical steels with high Nb-content is to atomize an Nb-containing melt without carbon. The carbon is subsequently added after atomization in the form of graphite-powder. The formation of NbC and the carbonization of the metal matrix are achieved during hot isostatic pressing (HIP) by diffusion. However, this process is complex and not applicable for large-scale industrial implementation.

### Summary

According to an aspect of the disclosure a powder-metallurgical steel consists of a steel composition, in % in weight: C: 0.35% to 0.6%, N: 0.01% to 0.3%, Cr: 12% to 15%,

Mo: 3% to 5.5%, Co: 1.6% to 5%, Nb: 1.2% to 1.75%, and optionally one or more of Si: less than 1.5%, Mn: less than 1.5%, W: less than 0.5%, Ni: less than 0.5%, Al: less than 0.3%, V: less than 1.0%, Ti: less than 1.0%, Ta: less than 0.5%, the balance being Fe and incidental impurities.

According to another aspect of the disclosure, a hardened powder-metallurgical steel comprises the powder-metallurgical steel recited above after having been subjected to a hardening process and a tempering process, the hardening process comprising heating the powder-metallurgical steel to a temperature between 1000°C and 1150°C followed by rapid cooling, and the tempering process comprising heating the cooled powder-metallurgical steel to a tempering temperature in a range between 200°C and 600°C, wherein the tempering is repeated at least once.

According to another aspect of the disclosure, a method of manufacturing a powder-metallurgical steel comprises melting a steel composition consisting of, in % in weight: C: 0.35% to 0.6%, N: 0.01% to 0.3%, Cr: 12% to 15%, Mo: 3% to 5.5%, Co: 1.6% to 5%, Nb: 1.2% to 1.75%, and optionally one or more of Si: less than 1.5%, Mn: less than 1.5%, W: less than 0.5%, Ni: less than 0.5%, Al: less than 0.3%, V: less than 1.0%, Ti: less than 1.0%, Ta: less than 0.5%, the balance being Fe and incidental impurities. The melted steel composition is then atomized to obtain a metal powder. The metal powder is hot isostatic pressed to obtain a powder-metallurgical steel product. The powder-metallurgical steel product is formed.

According to another aspect of the disclosure, a method of manufacturing a hardened powder-metallurgical steel further comprises hardening the powder-metallurgical steel product recited above by heating the powder-metallurgical steel product to a temperature between 1000°C and 1150°C followed by rapid cooling, and tempering the hardened powder-metallurgical steel product by heating the cooled powder-metallurgical steel product to an tempering temperature in a range between 200°C and 600°C, wherein the tempering is repeated at least once.

### Brief description of the drawings

The features of the various illustrated examples can be combined unless they exclude each other and/or can be selectively omitted if not described to be necessarily required. Examples are depicted in the drawings and are exemplarily detailed in the description which follows.
Figure 1 is an illustration of an exemplary manufacturing route of a powder-metallurgical steel according to the disclosure.
Figure 2 is a schematic illustration of exemplary processes of stress relief heating, hardening and tempering a powder-metallurgical steel according to the disclosure.
Figure 3 is a diagram illustrating a size distribution of NbC and NbCN primary carbides in the microstructure of an example of a powder-metallurgical steel according to the disclosure after hardening and tempering.
Figure 4 is a diagram showing a tempering curve of a hardened powder-metallurgical steel according to the disclosure as a function of the tempering temperature.
Figure 5 is a Schaeffler diagram illustrating the microstructure of the metal matrix of steel dependent on the Cr-equivalent and the Ni-equivalent of alloying elements, and further showing the microstructure of an example of a powder-metallurgical steel according to the disclosure after hardening and before tempering.
Figure 6 is a diagram showing the hardness and the impact toughness of an example of a powder-metallurgical steel according to the disclosure and an example of a commercially available powder-metallurgical steel after hardening and low temperature tempering and after hardening and high temperature tempering.
Figure 7 is a diagram showing the corrosion resistance of the examples of powder-metallurgical steels of Figure 6.

### Detailed description

In the powder-metallurgical steel according to the disclosure, Cr-rich carbides have been substituted with primary carbides such as NbC and NbCN (in the following written as "NbC(N)"). As the solubility of Cr in these monocarbides is low, Cr remains dissolved in the metal matrix and thus increases the corrosions resistance of the steel.

In other words, Nb causes the formation of primary carbides NbC(N) during atomization. The primary carbides consume C, resulting in very few Cr-rich carbides (e.g. Cr₇C₃ and Cr₂₃C₆) being formed during atomization and hot isostatic pressing. As a result, most of Cr remains in the metal matrix. The high Cr content in the metal matrix, together with a high Mo content, results in the desired corrosion resistance.

Further, it has been found that the addition of Co in a certain ratio to the Nb content is helpful to alleviate the problem of nozzle clogging and to improve the hardness of the powder-metallurgical steel.

Table 1 provides the chemical composition in % in weight of the powder-metallurgical steel according to the disclosure.

**Table 1: Chemical composition (in wt%) of steel melt according to the present disclosure**

| | **C** | **N** | **Si** | **Mn** | **Cr** | **Mo** | **W** | **Ni** |
|---|---|---|---|---|---|---|---|---|
| **Upper limit** | 0.60 | 0.30 | 1.5 | 1.5 | 15 | 5.5 | 0.50 | 0.50 |
| **Pref. upper limit** | 0.60 | 0.25 | 1.2 | 1.2 | 14 | 5.0 | 0.40 | 0.40 |
| **Spec. pref. upper limit** | 0.52 | 0.20 | 1.0 | 1.0 | 13.8 | 4.2 | 0.30 | 0.30 |
| **Spec. pref. lower limit** | 0.45 | 0.10 | 0.4 | 0.4 | 12.8 | 3.8 | 0 | 0 |
| **Pref. lower limit** | 0.40 | 0.05 | 0.20 | 0.20 | 12.5 | 3.5 | 0 | 0 |
| **Lower limit** | 0.35 | 0.01 | 0 | 0 | 12 | 3 | 0 | 0 |

**Table 1: (continuation)**

| | **Al** | **Co** | **Nb** | **V** | **Ti** | **Ta** | **Nb/Co** |
|---|---|---|---|---|---|---|---|
| **Upper limit** | 0.30 | 5 | 1.75 | 1.0 | 1.0 | 0.5 | |
| **Pref. upper limit** | 0.20 | 4 | 1.70 | 0.7 | 0.5 | 0.4 | |
| **Spec. pref. upper limit** | 0.10 | 3 | 1.65 | 0.5 | 0.2 | 0.3 | 0.85 |
| **Spec. pref. lower limit** | 0 | 1.95 | 1.4 | 0 | 0 | 0 | 0.50 |
| **Pref. lower limit** | 0 | 1.8 | 1.3 | 0 | 0 | 0 | |
| **Lower limit** | 0 | 1.6 | 1.2 | 0 | 0 | 0 | |

### Effects of the alloying elements

The effects of the alloying elements in relation to their content are described below. Percentages given below are % in weight (wt%). The balance of the chemical composition are Fe and incidental impurities.

### Carbon [C]

Carbon is essentially used to set the desired hardness. At least 0.35% of C is needed. However, the carbon content should not be too high, as this can lead to an excessively high proportion of precipitates in the form of carbides, which could have a negative effect on toughness and fatigue strength. Therefore, the upper limit is set to 0.6%.

### Nitrogen [N]

Next to Carbon, Nitrogen is the second most significant element contributing to the high achievable hardness level when dissolved interstitially. Additionally, it forms nitrides and carbonitrides with elements such as niobium or vanadium. To achieve these effects, a lower nitrogen limit of 0.01% is required. An upper limit of 0.3% is set because excessive nitrogen content stabilizes austenite, potentially resulting in high amounts of retained austenite.

### Silicon [Si]

Si is a solid solution strengthener and not a carbide-forming element, but influences carbide precipitation kinetics in steel. It shifts the formation of secondary hardening carbides to higher tempering temperatures, at which the non Cr-rich secondary hardening carbides M₇C₃ and M₂₃C₆ preferentially form. Si serves as a deoxidizing agent and is therefore present in low concentrations in almost all steels due to the manufacturing process. It increases the resistance to scaling, the yield strength and the tensile strength without significantly reducing the elongation. However, an excessively high Si content can significantly reduce toughness. Therefore, the upper limit is set to 1.5%. If Si is used as an alloying element, lower limits may, e.g., be set to 0.05%, 0.10%, 0.15%, 0.20%, 0.25%, 0.30%, 0.35%, 0.40%, 0.45%, 0.50%, 0.55%, or 0.60%.

### Manganese [Mn]

Mn can influence the hardness of the steel. In addition, Mn acts as a solid solution strengthener similar to Si. Mn increases the hardness, but too high a proportion can lead to a reduction in toughness. Therefore, the upper limit is set to 1.5%. If Mn is used as an alloying element, lower limits may, e.g., be set to 0.05%, 0.10%, 0.15%, 0.20%, 0.25%, 0.30%, 0.35%, 0.40%, 0.45%, 0.50%, 0.55%, or 0.60%.

### Chromium [Cr]

Cr leads to corrosion resistance in the metal matrix at a content greater than 12%. Therefore, the lower limit is set to 12%. It also leads to the desired solid solution strengthening. In general, Cr reduces the critical cooling rate and thus increases hardenability. Furthermore, increased Cr contents can lead to carbide precipitation and thus increase the hardness. Excessively high Cr contents can therefore also lead to negative effects in terms of toughness. In addition, excessive Cr content can have a negative effect on the retained austenite content after hardening, which may become too high. Therefore, the upper limit is set to 15%.

### Molybdenum [Mo]

Mo forms special carbides and, on the other hand, mixed carbides with iron. These are of the type M₂C and M₆C. The addition of Mo increases the activation energy for C diffusion in the austenite and thus lowers the diffusion coefficient for C and thus C diffusion. On the other hand, the addition of Mo leads to a refinement of the microstructure, i.e. a fine microstructure prevails regardless of the cooling rate (0.1°C/s to 60°C/s) during hardening. Grain coarsening remains low due to the low dissolution rate and the high dissolution temperature of the carbides (carbides counteract grain coarsening). This means that austenitizing (solution tempering) at higher hardening temperatures can achieve improved tempering resistance, as more carbide-forming elements can be precipitated and thus more carbides are formed. The hard carbides also increase the hot yield strength and wear-resistance. At high operation temperatures, Mo improves the scale resistance of the steel. Too high a content impairs machinability and, if Mo remains dissolved in the metal matrix, thermal conductivity. It could also happen that embrittlement occurs during tempering due to the formation of carbide precipitates at the former austenite grain boundaries. Therefore, the upper limit according to the disclosure is 5.5% by weight, preferably 5% by weight, particularly preferably 4.2% by weight. For the above-mentioned reasons, the lower limit according to the invention is 3% by weight, preferably 3.5% by weight, particularly preferably 3.8% by weight.

### Nickel [Ni]

Ni is an austenite-stabilizing element. Therefore, the upper limit is set to 0.5%.

### Cobalt [Co]

Co is an austenite-stabilizing element. It does not form carbides, but remains dissolved in the metal matrix and thus influences carbon diffusion. This leads to an increase in hot hardness (hardness at temperatures higher than room temperature to about 600°C) and improved toughness. Further, Co promotes the formation of secondary hardening carbides, as Co acts as nucleation site during tempering. This may increase the hardness caused by secondary hardening carbides (to an extent depending on the tempering temperature). An upper limit is determined due to saturation of carbide precipitation.

### Niobium [Nb]

Due to its high affinity to C, Nb is one of the strongest carbide-forming elements. It forms fine and evenly distributed precipitates of the monocarbide (MC) type, namely NbC(N). These are preferred due to their higher thermal resistance and higher hardness compared to other carbide types. This results in an increase in high-temperature strength, an increase in yield strength, wear resistance and an improvement in tempering resistance. However, at higher concentrations, a higher hardening temperature is required to dissolve the thermally stable, primary carbides NbC(N). High amounts of NbC(N) reduce toughness as well as polishability. Therefore, a lower limit of 1.2% and an upper limit of 1.75% are set.

### Vanadium [V]

V is a MC-forming element similar as Nb. However, an advantage of Nb over V is its low solubility in the metal matrix, which means that the NbC(N) content in the steel can be adjusted very precisely (and more precisely than the VC(N) content). Therefore, the upper limit is set to 1.0%, preferably to 0.70 especially preferably to 0.5%.

### Titanium [Ti]

Ti is a MC-forming element similar as Nb or V. However, in N-alloyed steels it causes the formation of coarse TiN, which is detrimental to toughness. Therefore, the upper limit is set to 1.0% preferably to 0.5%, especially preferably to 0.2%.

### Aluminum [Al]

Al acts as a deoxidizing agent and may optionally be added up to 0.3%.

### Tungsten [W]

W is a ferrite-stabilizing element. It is a strong carbide-former and is used to increase wear resistance. The addition of W improves the hot hardness and tempering resistance, which is why it is used as an additive in high-speed steel and hot-work tool steel. However, W is also a cost-intensive alloying element. It may optionally be added up to 0.5%.

### Nb/Co ratio

It was found that the Nb/Co ratio affects the prevention of nozzle clogging during atomization and can improve the hot hardness and other properties of the powder-metallurgical steel. Further, since there is an optimum amount of primary carbides NbC(N) to obtain high hardness (if there are too few primary carbides NbC(N), wear resistance and hardness deteriorate, but if there are too many primary carbides NbC(N), the metal matrix is depleted of C, causing the hardness of the metal matrix and also the overall hardness of the powder-metallurgy steel to decrease), carbon diffusion, which depends on the Co content, and the ability of Co to form nucleation sites for secondary hardening carbide formation, are important to achieve the optimum amount of primary carbides NbC(N) formation and secondary hardening carbides formation. Therefore, the Nb/Co ratio is preferably set to a range from 0.4 to 1.0 and more preferably to a range from 0.50 to 0.85.

### Manufacturing process

Figure 1 illustrates exemplary stages of a process of manufacturing a powder-metallurgical steel according to the disclosure.

At S1, a steel composition consisting of the elements of Table 1, the balance being Fe and incidental impurities, is melted by heating.

At S2, the Nb- and C-containing melt is atomized. For example, nitrogen may be used as an atomizing gas. Atomization of the melt produces steel particles (powder) of a size equal to or smaller than 350 pm, for example. During atomization, the particles solidify behind the nozzle. A cooling rate equal to or more than 1000 °C/s can be achieved.

When Nb- and C-containing melts are atomized, primary carbides NbC(N) are formed. These primary carbides tend to accumulate in the nozzle and clog it. However, as mentioned above, given the chemical composition of the melt, it was possible to atomize the melt without clogging the nozzle if the formation of the primary carbides NbC(N) was less than 3 vol% of the microstructure of the steels.

At S3, the metal powder is filled into a capsule which is then evacuated and sealed by welding, for example.

At S4, the metal powder is hot isostatic pressed to obtain a powder-metallurgical steel product. Hot isostatic pressing (HIP) may be carried out at a temperature between 1000°C and 1200°C and under a pressure of, e.g., 800 bar to 1200 bar. The HIP process may be carried out for 5 to 10 hours, for example. That way, the metal powder is converted into the powder-metallurgical steel product. In contrast to, e.g., a sintering process, in which only the surfaces of the particles are bonded, the powder-metallurgical steel product is homogeneous and free of any residual particle structure.

Differently put, the HIP process allows to produce a powder-metallurgical steel product which has a highly homogenous microstructure with very finely distributed primary carbides NbC(N) in the metal matrix. As a result, a high proportion of finely distributed primary carbide can be achieved in the powder-metallurgical steel product, which would not be possible without powder-metallurgical steel production.

At S5, the powder-metallurgical steel product may be formed by, e.g., forging or rolling. The forming temperature may be in a range between 1050°C and 1150°C. The degree of forming may, e.g., be equal to or more than 3 or 4. Thus, a change of the cross-sectional shape of a factor more than 3 or 4 may be obtained. This may mean that a main surface of the powder-metallurgical steel product of size A is reduced to a main surface of size A/3 or A/4, respectively.

At S6, the powder-metallurgical steel product may, e.g., be subjected to a heat treatment. The the heat treatment is used to soften the steel product. After heat treatment, the steel product is slowly cooled to prevent martensite formation (hardening).

At S7, the steel product can optionally be machined (e.g. by milling, grinding, polishing or another metalworking process) to give it a desired shape and/or surface finish.

The powder-metallurgical steel (also referred to as steel product) may then be sold to a customer, for example. The following production stages relate to subsequent processing of the powder-metallurgical steel as produced after some or all of the process stages S1 to S7. This subsequent processing may (optionally) be carried out by the customer and not by the steel manufacturer, for example. In other examples, the subsequent processing is carried out by the steel manufacturer.

Referring to Figure 2, before hardening at S9, the powder-metallurgical steel may, e.g., be subjected to a stress relief heat treatment at S8. For example, the stress relief heat treatment may be conducted at a temperature above 700°C, for example at a temperature of about 750°C. The stress relief heat treatment S8 reduces stress in the metal matrix.

The hardening treatment at S9 includes heating the powder-metallurgical steel to a temperature in the austenite phase region between 1000°C and 1150°C followed by rapid cooling. Hardening may comprise a certain holding time at the maximum temperature (hardening temperature). For example, the holding time may, e.g., be between 0 to 2 hours, in particular between 10 min and 1 hour.

Following the heat treatment, hardening further includes rapid cooling. Rapid cooling causes the transition of the austenitic matrix into fresh martensite and retained austenite. As indicated in Figure 2, by using a cooling medium such as, e.g., oil, gas, water or a polymer solution, the cooling rate may be substantially higher than under ambient atmosphere (dash-dotted line).

As already mentioned, the primary carbides, among them NbC(N), were formed during atomization. During hardening, the concentration of primary carbides is set. The primary carbides are partially dissolved depending on the hardening temperature. The higher the hardening temperature, the more primary carbides, among them NbC(N), are dissolved, i.e. they disappear.

The partial dissolution of the primary carbides during hardening results in the steel matrix being alloyed by the corresponding metal elements. In particular, the dissolution of Cr-rich primary carbides (which, however, have already largely been substituted by the primary carbides NbC(N)) increases the corrosion resistance of the steel.

After hardening, the primary carbides NbC(N) may have a fraction in volume in a range between 2 vol% and 5 vol%, in particular 2 vol% and 3.5 vol% of the hardened powder-metallurgical steel.

Figure 3 is a diagram showing a size distribution of the primary carbides NbC(N) contained in the metal matrix of a powder-metallurgical steel after hardening and tempering. Figure 3 shows the size distribution of NbC(N) in terms of the surface area coverage fraction in % versus ECD (Equivalent Circular Diameter) for two measurements (Measurement 1 and Measurement 2) at different locations of the same steel sample. Obviously, the mean size (mean ECD) of the NbC(N) primary carbides is smaller than 0.5 pm, 0.45 pm, 0.4 pm, 0.35 µm or 0.3 µm. A maximum size of less than 0.70 µm was observed in all ECD distributions. Due to the small size of the primary carbides, the steel has a high polishability, i.e. can be polished very well.

The steel product had a martensitic microstructure with about 3 vol% primary carbides NbC(N).

The (maximum) temperature of the hardening treatment sets the grain size and the amount or fraction in volume of the primary carbides NbC(N) in the steel. In other words, the ECD distribution of the primary carbides NbC(N) (see Figure 3) may be modified by the hardening process. Increasing the hardening temperature shifts the maximum of the ECD distribution towards smaller grain sizes (smaller ECD).

Further, the (maximum) temperature of hardening may be used to affect the PREN (Pitting Resistance Equivalent Number) of the powder-metallurgical steel after hardening.

Optionally, after rapid cooling to room temperature, cooling may be continued to temperatures below 0°C, in particular below -50°C or -80°C or -196°C (not shown). Deep cooling may comprise a certain holding time at the minimum temperature. For example, the holding time may, e.g., be between 0 to 4 hours, in particular 1 to 3 hours. Deep cooling to temperatures below 0°C is effective in reducing retained austenite in the metal matrix. This increases the hardness of the hardened powder-metallurgical steel.

After hardening, the powder-metallurgical steel product is tempered at S10. Tempering includes heating the powder-metallurgical steel product to a tempering temperature in a range between 200°C and 600°C. In particular, a preferred temperature range for tempering is between 300°C and 600°C, preferably between 400°C and 600°C and in particular between 450°C and 580°C. Tempering temperatures in a range between 480°C to 560°C may be particularly preferred.

As shown by way of example in Figure 2, the tempering process at S10 is repeated at least once. For example, three tempering cycles are used. Each tempering cycle may reach any of the temperatures mentioned above.

Further, each tempering cycle may comprise a certain holding time at a maximum temperature, e.g. at the tempering temperature. For example, the holding time may, e.g., be between 0 to 4 hours, in particular 1 to 3 hours.

During tempering, secondary hardening carbides are formed if the tempering temperature exceeds approximately 300°C. The formation of secondary hardening carbides M₇C₃, M₆C, M₂₃C₆ and M₃C, among them the chromium carbides Cr₇C₃ and Cr₂₃C₆, changes the properties of the hardened powder-metallurgical steel, in particular its hardness, toughness and corrosion resistance (the latter is determined by the corrosion resistance of the metal matrix, which is mainly based on the Cr and Mo content of the metal matrix).

Further, tempered martensite is formed by tempering. In this disclosure, martensite means fresh martensite and tempered martensite. Fresh martensite refers to martensite which is not tempered and which is formed during hardening. Tempered martensite is tempered during a tempering cycle.

In other words, fresh martensite means matensite after hardening. Martensite means fresh + tempered martensite.

### Low Temperature Tempering (LTT)

According to one embodiment, the tempering temperature is in a range between 200°C and 350°C, in particular between 200°C and 300°C or 200°C and 250°C. The stress in the martensite is reduced with the effect that the toughness of the steel is increased. Very few secondary hardening carbides M₇C₃, M₆C, M₂₃C₆ and M₃C to improve the hardness are formed during LTT. Consequently, more Cr and Mo remain in the metal matrix. Therefore, the hardened and low temperature tempered powder-metallurgical steel is highly corrosion resistant.

Since very few or no secondary hardening carbides are formed, the low temperature tempered steel has not such a high hardness as the high temperature tempered steel (see below). That is, during LTT, for example, the fraction in volume of secondary hardening carbides M₇C₃, M₆C, M₂₃C₆ and M₃C in the hardened powder-metallurgical steel may, e.g., be equal to or less than 1 vol%.

### High Temperature Tempering (HTT)

High temperature tempered steel is defined herein as a steel which has been tempered at temperatures above 450°C, for example at temperatures in a range between 450°C and 600°C or between 480°C and 560°C. At these temperatures, secondary hardening carbides M₇C₃, M₆C, M₂₃C₆ and M₃C, among them the chromium carbides Cr₇C₃ and Cr₂₃C₆, are formed. Further, temperatures above 450°C are needed to reduce the fraction in volume of retained austenite in the metal matrix.

The upper temperature limit of 600°C is given since above this temperature, carbides coarsen and hardness decreases. Due to the formation of secondary hardening carbides, in particular Cr-containig carbides, the metal matrix becomes increasingly depleted of Cr. Therefore, the corrosion resistance is lower than for low temperature tempered steels. However, tempering in the HTT temperature range may provide the best combination between hardness, toughness and still sufficient corrosion resistance, and may therefore be preferred for many applications.

The effect of tempering temperature on hardness is shown in Figure 4. The curve shows a typical behavior for steels that form secondary hardening carbides. In general, hardness decreases with increasing tempering temperature without the formation of secondary hardening carbides (see the low temperature section of the curve). At tempering temperatures above 300°C, the formation of the secondary hardening carbides begins. As can be seen from Figure 4, the hardness of the hardened powder-metallurgical steel product then increases with increasing tempering temperature.

After HTT, the fraction in volume of carbides (e.g. primary carbides such as NbC(N) and secondary hardening carbides, among them Cr₇C₃, Cr₂₃C₆) may be equal to or less than 15 vol%. For example, a fraction of primary carbides NbC(N) may be in a range between 1 and 5 vol%. The hardened powder-metallurgical steel after HTT may comprises a fraction in volume of less than 12.0 vol%, in particular less than 10.0 vol% of secondary hardening carbides M₇C₃, M₆C, M₂₃C₆ and M₃C. Specifically, a fraction in volume of Cr₇C₃ and C₂₃C₆ may be equal to or less than 5 vol%.

### Metal matrix microstructure

The metal matrix microstructure of the hardened powder-metallurgical steel for an example Ex_1 (compare Table 2 for the chemical composition) of the disclosure is shown in Figure 5. Figure 5 shows a Schaeffler diagram in which the Cr-equivalent and the Ni-equivalent represent the X-axis and the Y-axis, respectively. The Schaeffler diagram is divided into different areas that represent the microstructure present.

The Cr-equivalent represents the effectiveness of the ferrite-forming elements and is given by their mass fractions as Cr-equivalent = %Cr+%Mo+1.5%Si+0.5%Nb+2%Ti. The Ni-equivalent is calculated from the mass fractions of the alloying elements that cause iron to contain austenite in its structure, and is calculated as Ni-equivalent = %Ni+30%C+0.5%Mn+30(%N-0.02).

As apparent from Figure 5, the example Ex_1 is in the microstructure area "Austenite + Martensite". No ferrite fraction is present. The Cr-equivalent is 15 and the Ni-equivalent is 10.

It is to be noted that the Cr-equivalent and the Ni-equivalent exclusively rely on the elements of the metal matrix. Precipitations, such as, e.g., carbide precipitations, are not part of the metal matrix. Therefore, the Cr-equivalent of example Ex_1 would be 18 if computed based on the chemical composition of example Ex_1 (see Table 2). Analogously, the Ni-equivalent would be 19, if computed based on the chemical composition of example Ex_1. These calculations were done using the thermodynamic simulation software "Thermocalc 2024a with database TCFE7".

Regarding strength and wear resistance, an upper limit of the C and/or N content is given by the austenite stability (no martensite forms in the "Austenite" area). The C and/or N content is limited downwards by low martensite hardness and an insufficient fraction in volume of carbides or carbonitrides.

Regarding corrosion resistance, an upper limit of the Cr-content is given due to the stability range of ferrite and austenite. A lower limit is given by about 11 % free Cr in the metal matrix to ensure the required minimum corrosion resistance.

In general, after hardening and tempering, the fraction in volume of martensite (fresh + tempered martensite) in the metal matrix may be equal to or greater than 65 vol% or 70 vol% or 75 vol% or, more preferably, 80 vol% or 90 vol%. The fraction in volume of retained austenite after hardening and tempering may be equal to or less than 15 vol%, more preferably equal to or less than 10 vol%.

### Examples

Table 2 shows the chemical composition of example Ex_1 of a powder-metallurgical steel in accordance with the disclosure.

Examples Ex_2(ref.), Ex_3(ref.) and Ex_4(ref.) are reference examples.

**Table 2: Chemical compositions (in wt%) of a steel melt example Ex_1 according to the present disclosure and reference examples Ex 2(ref.), Ex 3(ref.), Ex_4(ref.)**

| **Examples** | **C** | **N** | **Si** | **Mn** | **Cr** | **Mo** | **W** | **Ni** |
|---|---|---|---|---|---|---|---|---|
| **Ex_1** | 0.51 | 0.15 | 0.43 | 0.42 | 12.9 | 3.9 | <0.05 | 0.03 |
| **Ex_2(ref.)** | 0.47 | 0.14 | 0.30 | 0.50 | 13.2 | 3.7 | <0.05 | 0.03 |
| **Ex_3(ref.)** | 0.52 | 0.16 | 0.35 | 0.48 | 13.0 | 4.1 | <0.05 | 0.03 |
| **Ex_4(ref.)** | **1.93** | 0.2 | 0.6 | 0.29 | **19.13** | **0.92** | **0.53** | 0.23 |

**Table 2: (continuation)**

| **Examples** | **Al** | **Co** | **Nb** | **V** | **Ti** | **Ta** | **Nb/Co** |
|---|---|---|---|---|---|---|---|
| **Ex_1** | 0.01 | 1.95 | 1.45 | <0.02 | 0.033 | <0.02 | 0.74 |
| **Ex_2(ref.)** | 0.02 | 1.45 | **2.10** | <0.02 | 0.035 | <0.02 | 1.45 |
| **Ex_3(ref.)** | 0.01 | 2.7 | **1.00** | <0.02 | 0.038 | <0.02 | 0.37 |
| **Ex 4(ref.)** | 0.005 | **0.05** | **0.005** | 3.96 | 0.005 | <0.02 | 0.1 |

In Table 2, the composition values that lie outside the ranges of Table 1 are printed in bold. In reference example Ex_2(ref.), too much Nb is present. There is too little Nb in reference example Ex_3(ref.). Reference example Ex_4(ref.) is not based on the concept underlying the disclosure, inter alia since too much Cr and too little Nb is used.

Examples Ex_1, Ex_2(ref.) and Ex_3(ref.) were produced by a process according to Figure 1 (stages S1 to S7). Subsequently, these powder-metallurgical steels were hardened and tempered (see Figure 2, S9 and S10).

### Hardening

Ex_1, Ex_2(ref.) and Ex_3(ref.) were hardened at 1130°C in a chamber furnace. The holding time was 0.5 hours. Rapid-cooling was carried out in oil down to room temperature. Alternatively, water, a polymer solution or pressurized N₂ could be used as a cooling medium. In addition, the examples were cooled down to -80°C, with a holding time of 2 hours.

After hardening and before tempering, the steel of Ex_1 had a mainly martensitic microstructure with retained austenite and about 3 vol% NbC(N).

Example Ex_4(ref.) was hardened at 1150°C in a vacuum furnace with a holding time of 0.5 hours. Rapid cooling down was carried out in N₂ at a pressure of 6 bar. This so-called vacuum tempering prevents the surface form scaling.

### Tempering

Two different tempering processes were applied, namely low temperature tempering (LTT) and high temperature tempering (HTT) .

Examples Ex_1, Ex_2(ref.) and Ex_3(ref.) were tempered as follows:
- LTT: two tempering cycles were carried out, each at 300°C and at a holding time of 2 hours.
- HTT: two tempering cycles were carried out, each at 520°C and at a holding time of 2 hours.

After hardening and tempering, the fraction in volume of the martensite (fresh martensite and tempered martensite) was equal to or greater than 79 vol%. The fraction in volume of NbC(N) and secondary hardening carbides was equal to or less than 13 vol% of the microstructure. The volume fraction of retained austenite was <10 vol.%.

For example Ex_4(ref.), high temperature tempering (HTT) and low temperature tempering (LTT) were carried out as follows:
- LTT: two tempering cycles were carried out, each at 200°C and at a holding time of 2 hours.
- HTT: two tempering cycles were carried out, each at 540°C and at a holding time of 2 hours.

Further, it is to be noted that the samples of Ex_4(ref.) for LTT were cooled down to -80°C, with a holding time of 2h, at the end of the hardening process. In contrast, the samples for HTT were not cooled below room temperature before tempering.

### Measurement result

Table 3 shows the mechanical properties and corrosion resistance properties of the examples as obtained by measurements.

The hardness was determined in units of HRc according to ASTM E 18-24, Rev. 04 24. Toughness was determined as impact toughness in units of J according to SEP 1314, Rev. 04 90.

Corrosion test: Exposure test in 20% boiling acetic acid for 24 hours. Mass loss of the samples (in g) was determined and related to time (in h) and surface area of the samples (in m²). Sample geometry was 40mm x 15mm x 5mm, the surface was ground with 120 grit.

**Table 3: Mechanical and corrosion resistance properties of the examples**

| **Examples** | **Ex_1** | | **Ex_2(ref.)** | | **Ex_3(ref.)** | | **Ex_4(ref.)** | |
|---|---|---|---|---|---|---|---|---|
| **Tempering** | **LTT** | **HTT** | **LTT** | **HTT** | **LTT** | **HTT** | **LTT** | **HTT** |
| **Impact Toughness [J]** | 96.3 | 49.5 | 77.8 | 43.5 | 98.7 | 52.7 | 37 | 46 |
| **Hardness [HRc]** | 57.6 | 61.2 | 56.4 | 58.9 | 54.3 | 57.1 | 61 | 59 |
| **Mass Loss [g/m²h]** | 0 | 36.7 | 0 | 34.3 | 0 | 46.7 | 10 | 150 |

Impact toughness and hardness are illustrated in Figure 6. The columns indicate impact toughness, while the diamonds indicate hardness. Corrosion resistance in terms of mass loss is illustrated in Figure 7.

In example Ex_2(ref.), the steel is Nb-rich and Nb/Co = 1.45. More coarse carbides are formed and therefore, a lower toughness is obtained. There is less C in the metal matrix, and therefore, a lower hardness is reached. However, Ex_2(ref.) yields a good corrosion resistance as more Cr remains in the metal matrix. Co is no longer as effective because too much C is already bound from the metal matrix in the form of NbC(N).

In example Ex_3(ref.), the steel has a substantially lower content of Nb, and Nb/Co = 0.37. As a result, the hardness is lower because less primary carbides, in particular NbC(N), are formed. Even in the case of HTT, this cannot be compensated by secondary hardening carbides (although there is more C in the metal matrix, which in turn forms more Cr-rich secondary hardening carbides). This results in a worse corrosion resistance.

In example Ex_1 according to the disclosure, the steel has a ratio Nb/Co = 0.74. About this ratio has been found to be an optimum between primary carbide NbC(N) formation and remaining C in the metal matrix for formation of secondary hardening carbides, wherein the formation of secondary hardening carbides (nucleation sites) is promoted by Co.

As shown in Table 3, Ex_1(LTT) provides the best combination of mechanical properties (impact toughness, hardness) at highest corrosion resistance (mass loss = 0 g/m²h). Ex_1(HTT) provides the best combination of mechanical properties (impact toughness, hardness) at still good corrosion resistance (mass loss = 36.7 g/m²h). The combination of high resistance to wear (high hardness) and corrosion opens-up the possibility of applications in areas such as steels for plastic processing (e.g., mold plates, tool inserts, hot runners, gating systems for, e.g., injection molding or other plastic manufacturing tools, etc.), industrial cutting tools especially in the food industry and tools in the medical sector.

Although specific examples have been illustrated and described herein, it will be appreciated by those of ordinary skill in the art that a variety of alternate and/or equivalent implementations may be substituted for the specific examples shown and described without departing from the scope of the present invention. This application is intended to cover any adaptations or variations of the specific examples discussed herein. Therefore, it is intended that this invention be limited only by the claims and the equivalents thereof.

## Claims

1. A powder-metallurgical steel consisting of a steel composition, in % in weight:
C: 0.35% to 0.6%,
N: 0.01% to 0.3%,
Cr: 12% to 15%,
Mo: 3% to 5.5%,
Co: 1.6% to 5%,
Nb: 1.2% to 1.75%,
and optionally one or more of
Si: less than 1.5%,
Mn: less than 1.5%,
W: less than 0.5%,
Ni: less than 0.5%,
Al: less than 0.3%,
V: less than 1.0%,
Ti: less than 1.0%,
Ta: less than 0.5%, the balance being Fe and incidental impurities.

2. The powder-metallurgical steel of claim 1, wherein
Nb: 1.3% to 1.70 or 1.4% to 1.65%.

3. The powder-metallurgical steel of claim 1 or 2, wherein
Co: 1.8% to 4% or 1.95% to 3%.

4. The powder-metallurgical steel of any of the preceding claims, wherein 0.4 < Nb/Co < 1.0 or 0.5 < Nb/Co < 0.85.

5. The powder-metallurgical steel of any of the preceding claims, wherein Cr: 12.5% to 14% or 12.8% to 13.8%.

6. The powder-metallurgical steel of any of the preceding claims, wherein Mo: 3.5% to 5.0% or 3.8% to 4.2%.

7. The powder-metallurgical steel of any of the preceding claims, wherein Si: more than 0.30 or 0.4%.

8. A hardened powder-metallurgical steel, comprising the powder-metallurgical steel of any of the preceding claims after having been subjected to a hardening process and a tempering process, the hardening process comprises heating the powder-metallurgical steel to a temperature between 1000°C and 1150°C followed by rapid cooling, and the tempering process comprises heating the cooled powder-metallurgical steel to a tempering temperature in a range between 200°C and 600°C, wherein the tempering is repeated at least once.

9. The hardened powder-metallurgical steel of claim 8, comprising a metal matrix and primary carbides NbC and NbCN distributed in the metal matrix, wherein
a maximum of the equivalent circular diameter, ECD, distribution of the primary carbides NbC and NbCN is in a range between 0.05 µm and 0.4 pm, in particular between 0.1 µm and 0.35 µm and/or
the primary carbides NbC and NbCN have a total volume in a range between 2 vol% and 5 vol%, in particular 2 vol% and 3.5 vol% of the hardened powder-metallurgical steel.

10. The hardened powder-metallurgical steel of claim 8 or 9, wherein the tempering temperature is in a range between 200°C and 350°C, and the hardened powder-metallurgical steel comprises a hardness of equal to or more than 57HRc and an impact toughness of equal to or more than 90J.

11. The hardened powder-metallurgical steel of claim 8 or 9, wherein the tempering temperature is in a range between 450°C and 600°C, in particular 480°C and 560°C, and the hardened powder-metallurgical steel comprises a hardness of equal to or more than 60HRc and an impact toughness of equal to or more than 45J.

12. A method of manufacturing a powder-metallurgical steel, the method comprising:
melting a steel composition consisting of, in % in weight:
C: 0.35% to 0.6%,
N: 0.01% to 0.3%,
Cr: 12% to 15%,
Mo: 3% to 5.5%,
Co: 1.6% to 5%,
Nb: 1.2% to 1.75%,
and optionally one or more of
Si: less than 1.5%,
Mn: less than 1.5%,
W: less than 0.5%,
Ni: less than 0.5%,
Al: less than 0.3%,
V: less than 1.0%,
Ti: less than 1.0%,
Ta: less than 0.5%, the balance being Fe and incidental impurities;
atomizing the melted steel composition to obtain a metal powder;
hot isostatic pressing the metal powder to obtain a powder-metallurgical steel product; and
forming the powder-metallurgical steel product.

13. The method of claim 12, further comprising:
hardening the powder-metallurgical steel product by heating the powder-metallurgical steel product to a temperature between 1000°C and 1150°C followed by rapid cooling, and
tempering the hardened powder-metallurgical steel product by heating the cooled powder-metallurgical steel product to a tempering temperature in a range between 200°C and 600°C, wherein the tempering is repeated at least once.

14. The method of claim 13, wherein the tempering temperature is in a range between 200°C and 350°C, and the hardened powder-metallurgical steel after tempering comprises a fraction in volume of less than 1.0 vol% of secondary hardening carbides M₇C₃, M₆C, M₂₃C₆ and M₃C, wherein M denotes a metal element of the steel composition.

15. The method of claim 13, wherein the tempering temperature is in a range between 450°C and 600°C, in particular 480°C and 560°C, and the hardened powder-metallurgical steel after tempering comprises a fraction in volume of less than 12.0 vol%, in particular less than 10.0 vol% of secondary hardening carbides M₇C₃, M₆C, M₂₃C₆ and M₃C, wherein M denotes a metal element of the steel composition.
